

**1**

3,704,155

**THERMOGRAPHIC STENCIL SHEET AND  
METHOD OF MAKING AN IMAGED  
STENCIL SHEET**

Bror E. Anderson, Arlington Heights, and Margery L. Schick, Mount Prospect, Ill., assignors to Weber Marking Systems, Inc., Arlington Heights, Ill.  
No Drawing. Continuation-in-part of application Ser. No. 674,153, Oct. 10, 1967. This application Apr. 9, 1970, Ser. No. 27,135

Int. Cl. B41m 1/24

U.S. Cl. 117—35.5

10 Claims

**ABSTRACT OF THE DISCLOSURE**

A thermographic stencil sheet which may be imaged by heat generated by infrared ray absorption with but low oil transfer to an adjacent original includes an ink-pervious base sheet and an ink-impervious coating thereon of a heat-flowable composition of cellulose acetate butyrate film-forming material and plasticizing material partially but incompletely compatible with the film-forming material, the composition being characterized by forming a cooled melt having a defined pourable liquid volume, and the plasticizing material being characterized by defined tack and aniline point limits. The stencil sheet may be imaged by exposing an original in contact with the sheet to infrared radiation to generate heat in the image areas of the original sufficient to render the composition flowable in the image areas of the stencil sheet, and causing the composition to flow from the image areas to thereby form corresponding ink-transmitting openings in the stencil sheet.

**RELATED APPLICATION**

This is a continuation-in-part of application Ser. No. 674,153, filed Oct. 10, 1967.

**BACKGROUND OF THE INVENTION**

This invention relates to a thermographic stencil sheet of the type which includes a layer of a heat-flowable composition and to a method of making an imaged stencil sheet therewith by subjecting image areas of the stencil sheet to heat generated by infrared ray absorption.

Our copending U.S. patent application Ser. No. 674,153, filed Oct. 10, 1967 now abandoned, discloses a thermographic stencil sheet including an ink-pervious base sheet and an ink-impervious coating thereon of a heat-flowable composition of cellulose acetate butyrate film forming material and plasticizing material partially but incompletely compatible with the film-forming material. The stencil sheet is now in widespread commercial use. It is employed preferably in a stencil sheet assembly including a contacting absorbent sheet on one surface thereof, and a more rigid backing sheet on the opposite surface thereof and to which the absorbent sheet and the stencil sheet are mounted. In use, an original, such as a typed or printed sheet, is inserted between the stencil sheet and the backing sheet, and the assembly is exposed to infrared radiation on the face side of the absorbent sheet in a thermal copier such as a Thermo-Fax machine (3M Company). Heat is generated in the radiation absorptive graphic portions of the original to cause the stencil sheet composition to flow in corresponding areas and thereby produce corresponding image openings in the stencil sheet. The composition rendered flowable is absorbed by the absorbent sheet and/or adjoining areas of the stencil sheet. The original and the absorbent sheet are separated from the imaged stencil sheet, the stencil

**2**

sheet and the backing sheet are placed on a mimeograph duplicating machine followed by separation of the backing sheet, and the machine is operated to produce multiple mimeograph copies of the original.

It was found in use that "oil" was transferred from the stencil sheet to the original in the image areas. The oil frequently broadened and feathered the copy on the original (smudging) and the presence of oil on the original was not a desirable condition. The smudging of the original affected the imaging speed in subsequent exposures, owing to the broadening of the imaged characters or transfer from the original to the stencil sheet. Subsequent performance was affected when the original was removed from the file for rerun, or in the event that optimum exposure was not used in imaging the first stencil.

It would be desirable to reduce the oil transfer to acceptable limits while preserving the advantageous properties of the stencil sheet of our aforesaid copending application.

**SUMMARY OF THE INVENTION**

The present invention provides a thermographic stencil sheet of the type disclosed in our aforesaid copending application which exhibits low oil transfer while maintaining and in many cases improving on copy quality. The stencil sheet includes a heat-flowable composition characterized by forming a cooled melt having a defined pourable liquid volume, and a plasticizing material in the composition characterized by defined tack and aniline point limits.

More particularly the thermographic stencil sheet of the present invention comprises an ink-pervious base sheet, and an ink-impervious coating thereon of a heat-flowable composition of cellulose acetate butyrate film-forming material, and plasticizing material having (a) a tack index, as defined hereinafter, of at least about 10, and (b) a maximum mixed aniline point of about 110° F., the said composition initially forming a clear 35 homogeneous single phase melt at a maximum temperature of about 320° F. and forming a solid-liquid two-phase mixture when cooled from the melt to room temperature, at least one phase of the said mixture incorporating substantial proportions of both the film-forming material and the plasticizing material, the mixture having a pourable liquid volume which is a maximum of about one-fourth the volume of the solid phase, the said composition being soluble in a volatile solvent and forming a substantially clear homogeneous continuous im- 40 perforate coating when deposited from a solution thereof, and the said coating being provided on the base sheet by deposition of the composition on the base sheet from a solvent solution thereof, the melting point of the coating being in the range of about 150–320° F.

The invention also provides a method of making an imaged stencil sheet, wherein the thermographic stencil sheet is employed in contact with a graphic original, image areas of the stencil sheet are subjected to heat generated in the original by infrared ray absorption to render the composition flowable in the stencil sheet image areas, and the composition is caused to flow from the image areas and thereby form corresponding ink-transmitting image openings in the stencil sheet.

**DESCRIPTION OF THE PREFERRED  
EMBODIMENTS**

The thermographic stencil sheet includes a stencil base tissue sheet that may be formed of any suitable fiber, such as abaca and wood fibers, kozo fiber, or polyester fibers, loosely arranged to provide a foraminous, highly permeable tissue. The tissue may weigh about four and one-half to twelve pounds per 3,000 sq. ft. (24" x 36", 500 sheets).

A heat-flowable coating composition, which is solid at ambient temperature, is applied to the base sheet at a rate of about 14 to 24 lbs. (dry basis), preferably about 20 lbs. per 3,000 sq. ft. The coating composition melts in the range of about 150°-320° F., more preferably 200-300° F.

The heat-flowable coating composition includes cellulose acetate butyrate film-forming material, which is capable of forming a continuous, cohesive, flexible, ink-impermeable film. The film-forming material is plasticizable to melt in the range of about 150-320° F. The film-forming material is employed in a proportion in the range of about 8-50%, preferably about 8-30%, and more preferably about 14-23% by weight of the coating composition, including the film-forming and plasticizing materials and exclusive of additives thereto. The volume ratio of the film-forming material to the total plasticizing material in the coating composition preferably is in the range of about 1:13 to 1:3.5.

Of the available grades of cellulose acetate butyrate, it is preferred to employ those having values of about 35-55% butyryl content, more preferably above about 49%, and about 1.5-13% acetyl content, by weight. The hydroxyl content varies up to about 4.5% by weight, and it is preferred that the hydroxyl content be below about 0.4%. The viscosity is about 0.15-6 seconds, by A.S.T.M. Method D-1343-54T in Formula A, A.S.T.M. Method D-871-54T. The melting or softening points range from about 265 to 360° F.

The film-forming material is combined in the coating composition with a plasticizing material partially but incompletely compatible therewith. Such plasticizing material is defined to mean material which when heated with the film-forming material in the proportions used forms a clear homogeneous single phase melt, and which when cooled from the melt to ambient or room temperature forms a two-phase mixture, at least one phase of the mixture incorporating substantial proportions of both the film-forming material and the plasticizing material. The materials employed in the composition initially form a single phase melt at a maximum temperature of about 280-320° F., varying with the specific composition. Such temperature is referred to as the compatibility temperature of the composition. It is preferred that the compatibility temperature be at least about 120° F., and in further preferred embodiments of the invention, the compatibility temperature is above about 170° F.

Upon cooling below the compatibility temperature, the liquid separates into two phases. The mixture remains fluid over a temperature range, and then the phase containing the major proportion of the film-former gradually hardens to a solid as the coating cools to room temperature. The liquid phase may be trapped by the gel structure of the solid phase at room temperature, or it may separate into a discrete liquid component.

A characteristic of the present invention is that the foregoing mixture at room temperature has a maximum pourable liquid volume of about one-fourth the volume of the solid phase, and it is preferred that the pourable liquid volume be a maximum of about one-eighth the volume of the solid phase. For example, the mixture is cooled to room temperature with stirring, and its consistency is observed. A uniform gel or slush, having no solid separation, generally is optimum for low oil transfer. The mixture may separate into solid and liquid fractions, the solid being particulate or in the form of a ball, from which a liquid may be poured. It is the volume of such pourable liquid with reference to the solid content of the mixture which is referred to in connection with the above pourable liquid volume maximums.

The plasticizing material having partial but incomplete compatibility with the film-forming material may constitute a single plasticizer, or may include a plurality of plasticizers. The plasticizers are substantially non-volatile substances which serve to modify the physical

properties of the film-forming material, including the melting or softening point, compatibility, and/or flow properties. They may be either liquid or solid at temperatures from ambient temperature up to close to imaging temperature, but at least must be liquid when mixed with other plasticizers at imaging temperature.

The plasticizers generally fall into three groups as regards compatibility with the film-forming material: partially but incompletely compatible, incompatible, and compatible substances. Certain of the partially compatible plasticizers may be employed as sole plasticizers. Alternatively, two or more plasticizers having individual compatibilities varying from complete compatibility to complete incompatibility may be employed, so long as the plasticizers together provide the proper balance of compatibility with the film-forming material. When a plurality of plasticizers is employed, it is preferred that they be compatible with each other at room temperature, forming a single phase mixture after heating together and cooling.

The above-described characteristic composition having the defined maximum pourable liquid volume constitutes a relatively compatible composition. When such a composition is employed in the stencil coating, the coating may suffer from blocking, owing to tackiness accompanying increased compatibility. Blocking is a condition of adherence or sticking to adjacent stencil material in a roll, or sticking to the original or the top tissue during imaging, which causes pinholing. We have found that plasticizing material can be formulated on the basis of defined tack limits to minimize blocking. In particular, a plasticizing material, including one or more plasticizers, is employed which has a tack index of at least about 10, determined as follows:

35 The "Tack Rolling Ball Method" of the Pressure Sensitive Tape Council (Glenview, Ill.) was modified for a lower tack level, and the modified method is identified herein as the "modified rolling ball method." The apparatus included a glass plate, 8½" x 11" supported in horizontal position. A second glass plate, 3" x 6", was mounted with its 3" edge abutting the 8½" edge of the first plate, with their upper edges or corners in aligned contact with each other. A ball holder was affixed to the smaller plate to release a ball ½" from its outer end. 40 The outer end of the smaller plate was elevated so that the surface of the plate at the point of ball release was 0.203" above the horizontal plane of the upper surface of the large plate. The apparatus thus was arranged for releasing a steel ball on the small plate to roll down 5½" 45 of the small plate and on to the large plate. Steel balls were used having a diameter of 7/16" and weighing 5.48 grams.

In the test, a film of the plasticizing material to be tested is cast on the large plate and drawn down to a thickness of ½ mil. The film is cast at a temperature such as to render the plasticizing material sufficiently fluid, and is cooled, if necessary, for measurement at room temperature (77° F.). The cast film is drawn down with a rod or other suitable means to provide the film thickness of 55 ½ mil.

60 A ball rolling across the film will experience a decelerating force proportional to the velocity of the ball and the tackiness of the film. Liquid viscosity also has an effect, minimized by employing the very thin film. In addition, an experimentally determined viscosity factor is applied to the results.

Tack measurements are made in inches of ball roll on the larger plate bearing the film, measured to the point the ball stops. The tackier the material, the shorter the distance of ball roll. The tack index referred to herein and in the claims is determined by measurement of the amount of ball roll on the horizontal plate, in inches, multiplied by the  $\log_{10}$  of the viscosity of the plasticizing material in centipoises at 77° F. In the invention, such index is at least about 10.

5

The above-described conditions of maximum pourable liquid volume from a cooled melt of the composition of film-forming and plasticizing materials, and of a minimum tack index will in general serve to identify the coating compositions, both in their materials and in their relative proportions, which will provide low oil transfer with minimized blocking. There are, however, exceptions, and it is found in the invention that the exceptions noted are excluded by limitations on the aniline point of the plasticizing material, the aniline point serving as an indication of the compatibility of the plasticizing material with the film-forming material. Thus, the plasticizing materials employed in the invention are relatively compatible with the film-forming material, while remaining partially but incompletely compatible therewith. In general, a maximum mixed aniline point of about 110° F. is specified for the plasticizing material. In a specific embodiment of the invention, described hereinafter, it has also been found that oil transfer is reduced in the presence of an aluminum stearate gelling agent. In such case, the maximum mixed aniline point may be about 110-135° F.

Mixed aniline point as referred to herein and in the claims is determined by A.S.T.M. test D-1012-62. It is the minimum equilibrium temperature of a mixture of 2 volumes of aniline, 1 volume of sample, and 1 volume of n-heptane of specified purity. Straight aniline point is determined according to the A.S.T.M. test, and is the minimum equilibrium temperature of a mixture of 1 volume of aniline and 1 volume of sample. For formulating purposes, it is generally useful to mix high aniline point material with a low aniline point, low tack material such as Hercolube A (described hereinafter), in a 50:50 volume ratio, and run the aniline point of the mixture. Similarly, it is useful to mix low aniline point material with high aniline point material such as Mobilsol L (described hereinafter). Theoretical aniline points may be determined in this manner for materials which otherwise cannot be measured or can be measured only with difficulty. Theoretical aniline points referred to hereinafter were determined in the foregoing manner.

The plasticizing material and proportions thereof are selected on the basis of the herein-defined physical properties. Numerous and diverse materials may be employed, in a variety of combinations and relative proportions. Most frequently, a plurality of individual plasticizers are combined to achieve the specified physical conditions and optimum results. When the plasticizing material satisfies the basic conditions, the proportions of individual plasticizers thereof may be adjusted within the defined limits to achieve optimum properties.

The plasticizing material is oleaginous or oily in nature that is, it contains one or more oleaginous plasticizers. While numerous oleaginous plasticizers may be employed, it is presently preferred to employ one or more members selected from the group consisting of mineral oil, castor oil, hexadecyl alcohol, polypropylene glycol monobutyl ether, polyoxyethylene ethers or lanolin alcohols, pentaerythritol tetra-esters of aliphatic acids having from 5 to 10 carbon atoms, and trimethylol propane tri-esters of aliphatic acids having from 5 to 10 carbon atoms. An oleaginous plasticizer or mixture of plasticizers may be present in a proportion in the range of about 5-85% by weight of the film-forming material and plasticizing material, such materials being referred to herein as the active materials, excluding materials which are neither film-formers nor plasticizers, such as inert solids and other materials performing other functions.

It is further preferred to employ plasticizing material containing mineral oil, an ester of an aliphatic acid having from 5 to 10 carbon atoms, as described above, or a mixture of the two. The mineral oil preferably is employed in a proportion of about 5-70% by weight of the composition of film-forming material and plasticizing material, more preferably, 10 to 50%. The aliphatic acid ester is

6

employed in a proportion of about 5-85% by weight of the composition, preferably 15-55%.

A valuable class of plasticizers generally employed with one or more other plasticizers in the invention constitutes materials having a nucleus selected from the group consisting of



such materials provide low oil transfer and/or low tackiness properties. They may be employed in proportions of about 5-75%, preferably 15-55% by weight of the film-forming and plasticizing materials.

The materials having the foregoing nucleus include lanolin sterols, which serve to impart low tackiness.

The materials including such nucleus also include the acid constituents of rosin, known as resin acids, and their derivatives, including derivatives of the resin acids both in refined form and as present in rosin, about 90% of which constitutes resin acids. The resin acids are chiefly the abietic acid type, and abietic acid is the major constituent of the acids. The resin acid derivatives are preferred as having greater stability than the resin acids.

Preferred derivatives of the resin acids include hydrogenated resin acids, esters of hydrogenated resin acids, esters of resin acids, hydroabietyl alcohol, and esters of hydroabietyl alcohol. Preferred esters include the methyl, pentaerythritol, glycerol, phthalate, and polyol esters, the latter including particularly the diethylene and triethylene glycol esters. Such materials are in general relatively compatible with the film-forming material and with other plasticizers, and they serve to impart low oil transfer and/or better durability to the coating composition, partially as a result of the higher viscosity they impart.

A formulation for high viscosity may assist valuably in the provision of a low oil transfer composition. With higher viscosity, compatibility of the plasticizing material with the film-forming material may be and often preferably is reduced with the aniline point of the plasticizing material being higher. Also, the tackiness of the plasticizing material may be higher, and the pourable liquid volume from the cooled composition melt may be greater. However, the copy quality may suffer in some cases.

The film-forming and plasticizing materials of the coating composition are soluble in a volatile solvent and are selected and blended in proportions so as to form a substantially clear homogeneous continuous imperforate coating when deposited from a solution thereof, the coating then being provided on the base sheet by deposition of the composition thereon from such solution. In this connection, reference to clarity of the coating, as an index of compatibility, is to be understood as being exclusive of the effects of additives other than the active or basic film-forming and plasticizing materials, i.e., additives such as solids incorporated for other purposes, fillers and others. Reference to clarity is also exclusive of the opacifying effects of materials having an inherent opacity, such as waxy materials, and of the presence of materials which are solid at room temperature and are incorporated above their solubility limits at room temperature.

The coating composition preferably is completely soluble in a volatile solvent at a temperature below about 140° F., more preferably, at room temperature. The preferred coating compositions are soluble in organic solvent mixtures of aromatic hydrocarbons, and aliphatic esters and/or aliphatic alcohols, and are deposited on the base sheet from a solution therein by evaporation of

the solvent. The composition deposited in this manner forms a uniform gel on the base sheet, which is irreversibly physically altered when heated to its melting point.

The film-forming and plasticizing materials are selected and blended in proportions so as to form a stencil sheet coating melting in the range of about 150-320° F. The stencil coating may melt at a temperature from below to above the compatibility temperature, described above.

Reference to the melting point of the coating herein means the temperature at which a free film of coating on a vertical surface becomes liquid enough to flow. (A free film is obtained by depositing the coating from solvent onto a non-porous surface.)

For optimum results, it may be necessary to adjust the ingredients of the coating composition and their proportions on the basis of observed results. That is, adjustment may be made to improve uniformity, featheriness, and brokenness of the imaged characters, oiliness, blocking, speed of imaging, and durability. The majority of the stencil sheets illustrated herein may also be imaged mechanically, as by typing, which constitutes a substantial advantage. Adjustment of the materials and proportions also may be made to provide optimum typing sensitivity.

The stencil sheet may be imaged in a conventional thermographic machine, such as a roller-type copier as represented by Copy-Rite Model CF 8 (Polyfax Corporation), and a belt-type copier such as a Thermo-Fax Model 45CG "Secretary" machine. A tungsten filament lamp or other suitable source of infrared radiation is employed for imaging. A printed original in contact with the stencil sheet is exposed to radiation substantially instantaneously, i.e., on the order of about 0.03 to 0.1 second, to generate a temperature rise in the image portions of the original from about ambient temperature to a temperature sufficient to produce a temperature in the image portions of the stencil sheet in the range of about 150-320° F.

The coating composition in the stencil sheet is reduced to a flowable condition substantially instantaneously and is absorbed by the absorbent sheet or into adjacent areas of the stencil sheet immediately thereafter, to leave ink-transmitting image openings in the stencil sheet. The openings are bridged by the fibers of the stencil base sheet, which is ink-previous, and the base sheet fibers serve to retain letter centers and the like in place. The imaged stencil sheet is separated from the original and the absorbent sheet for use as a duplicating master.

An advantageous additive to the composition of film-forming and plasticizing materials satisfying the above conditions is a gelling agent for the plasticizing material, forming an irreversible gel upon heating up to about 210° F. Especially low oil transfer is achieved in this manner. This embodiment is preferably employed when the stencil is intended for use on roller type thermal copiers, whereas it is not well adapted for the belt-type copiers. It appears that the superiority of the roller type copiers is due to the good contact of the stencil with the original and the pressure exerted on the stencil at the time of imaging, serving to remove fluid from the image areas.

The preferred gelling agents are the aluminum stearates. While various grades will provide improvement, aluminum distearate of the type that gives highest gel strength is preferred. The stearates preferably are employed in a proportion of about 1-15%, preferably 8-11% by weight of the composition including film-forming and plasticizing materials, and stearate.

Employing an aluminum stearate gelling agent, the maximum mixed aniline point of the plasticizing material may be greater, in the range of about 110-135° F., increasing in said range with increasing proportion of the gelling agent. The use of the gelling agent also is more broadly applicable to other coating compositions within the scope of our application Ser. No. 674,153, inasmuch

as the pourable liquid volume and the tack index conditions no longer need be met.

In the examples which follow, the coating compositions were dissolved in one of several solvent mixtures, 5 identified as follows:

GRAMS OF SOLVENT PER 100 GRAMS ACTIVE MATERIALS

|    |                 | Ethyl<br>alcohol, 95%<br>denatured<br>(U.S. Gov't.<br>Formula C) | Ethyl<br>acetate,<br>99% |
|----|-----------------|------------------------------------------------------------------|--------------------------|
| 10 | Toluene         |                                                                  |                          |
| 15 | Solvent number: |                                                                  |                          |
| 1  | .....           | 92.8                                                             | 26.4                     |
| 2  | .....           | 116.5                                                            | 32.5                     |
| 3  | .....           | 115.0                                                            | 32.5                     |
| 4  | .....           | 113.7                                                            | 32.5                     |
| 5  | .....           | 103.0                                                            | 29.2                     |
|    |                 |                                                                  | 75.8                     |

The materials of each coating composition were dissolved at a concentration of about 30-35% by weight in the solvent mixture. The materials were mixed at room temperature, with a solution of the cellulose acetate butyrate being added last. Stencil base tissue sheet material made of abaca fiber was coated and impregnated with the solution. The tissue weighed 6.7 lbs. per 3,000 sq. ft. The sheet material was coated with the solution by passing it over a roll carrying the solution, removing excess fluid by a doctor rod, and drying with circulated air heated up to about 130° F. The total coated weight of the resulting stencil sheet ranged from 25.5 to 28 lbs. per 3,000 sq. ft. The thickness of the resulting stencil sheet was about 2 1/4 mils.

In addition to the listed ingredients, each coating composition included 0.17 gram of an antioxidant per 100 grams of active materials, the antioxidant being Carstab DLTDP, described hereinafter.

Each stencil sheet was assembled with an absorbent sheet for imaging tests. The absorbent sheet was 10 lb. per 2,880 sq. ft. tissue formed of mixed abaca and wood pulp fibers (Grade 55 tissue, Dexter Corporation). Oil transfer and image smudging was determined on carbon ribbon copy typed on bond paper and on offset printed stock. Blocking was determined by storing unassembled stencil sheets in contact with each other in foil, at room temperature. Blocking was also determined in most cases by evaluating pinholing upon exposure with a blank sheet of paper in a thermal copier. Durability was determined on a label printer type of mimeograph stencil duplicating machine.

Materials which may be employed in the invention, and referred to herein, are described as follows:

CAB 500-1 is cellulose acetate butyrate grade EAB 500-1 (Eastman Chemical Products) having an average butyryl content of 49.6%, an average acetyl content of 5.5%, a hydroxyl content of 0.15-0.36%, a viscosity of 0.8-1.2 seconds determined by the hereinabove-identified A.S.T.M. method, and a melting point range of about 329-347° F.

CAB 451-1 is cellulose acetate butyrate grade EAB 451-1 (Eastman Chemical Products) having an average butyryl content of 44%, an average acetyl content of 8.5%, an average hydroxyl content of about 1.3%, a viscosity of 1-2 seconds by the A.S.T.M. method, and a melting point range of 302-311° F.

Carstab DLTDP (Carlisle Chemical Works) is dilauryl thiodipropionate.

Mobilsol L (Socony Mobil Oil Co.) is a refined naphthenic petroleum oil having a viscosity of 61 Saybolt Universal Seconds (SUS) at 100° F., an aniline point of 165° F. (straight, A.S.T.M. test D-1012-62), an API gravity of 25.7°, and a distillation range of 490-708° F. (100%).

Compressor Lube 1500 (Witco Chemical Co.) is a 75 highly paraffinic white mineral oil having typical vis-

cosities of 1537 SUS at 100° F. and 95 SUS at 210° F., and a specific gravity of 0.886. Its aniline point is greater than 230° F. (straight).

Hercolube A (Hercules, Inc.) is the mono-pentaerythritol tetra-ester of capric acid, having an acid number of 0.1, a saponification number of 420, and a specific gravity of 1.002 at 25° C. Its mixed aniline point is 62° F.

MCP-42 (Mobil Chemical Co.) is a mixed tetra-ester of pentaerythritol and a mixture of aliphatic acids having 5-10 carbon atoms and an average carbon number of 6.9. The acids include 15-20% branched chain and the balance straight chain alcanoic acids. The specific gravity is 1.00 at 25° C. Its mixed aniline point is 42° F.

MCP-99 (Mobil Chemical Co.) is a mixed tri-ester of trimethylol propane and a mixture of aliphatic acids having 5-10 carbon atoms and an average carbon number of 8.3.

The acids are straight chain alcanoic acids. The specific gravity is 0.985 at 25° C. Its mixed aniline point is 58° F.

Ucon LB-70-X (Union Carbide) is polypropylene glycol monobutyl ether having a viscosity of 70 centipoises at 100° F. Its mixed aniline point is 77° F.

Ucon LB-300-X (Union Carbide) is polypropylene glycol monobutyl ether having a viscosity of 70 centipoises at 100° F. Its mixed aniline point is 102° F.

Solulan 5 (American Cholesterol Products) is a poly-oxyethylene ether of lanolin alcohols and contains lanolin sterols. It is a 5 mole ethylene oxide ether of the lanolin alcohols. It typically has an acid number of 3 max., a hydroxyl number of 120-135, a saponification number of 10 max., and an iodine value of 20-30. Its mixed aniline point is less than 40° F.

Modulan (American Cholesterol Products) is acetylated USP lanolin as described in U.S. Pat. No. 2,725,334. It typically has an acid number of 3 max., a hydroxyl number of 10 max., a saponification number of 95-125, and a melting range of 30-40° C. Its mixed aniline point is 131° F.

Acetulan (American Cholesterol Products) is a liquid fraction of acetylated lanolin alcohols typically having an acid number of 1 max., a hydroxyl number of 8 max., a saponification number of 180-200, an iodine number of 6-10, a specific gravity of 0.850-0.880 at 25° C., and a viscosity of about 10 centipoises at 25° C. Its mixed aniline point is 35° F.

Hercolyn D (Hercules, Inc.) is a hydrogenated methyl ester of rosin purified by steam distillation, a liquid having a Gardner-Holdt viscosity at 25° C. of Z2-Z3 and an acid number of 7. Its mixed aniline point is 58° F.

Abitol (Hercules, Inc.) is technical hydroabietyl alcohol having a viscosity of 200 centipoises at 80° C., a specific gravity of 1.008 at 25° C., a maximum acid number of 0.4, a maximum saponification number of 16, and a mixed aniline point of less than 40° F.

Cellolyn 21 (Hercules, Inc.) is a phthalate ester of technical hydroabietyl alcohol. It typically has an acid number of 8, a saponification number of 129, a specific gravity of 1.05 at 25° C., a softening point (Hercules drop method) of 65° C., and a mixed aniline point of 55° F.

Cellolyn 104 (Hercules, Inc.) is a pentaerythritol ester of rosin, typically having an acid number of 30, a specific gravity of 1.13 at 25° C., a softening point (Hercules drop method) of 101° C., and a mixed aniline point of 145° F.

Staybelite Ester 3 (Hercules, Inc.) is a triethylene glycol ester of hydrogenated rosin, typically having a viscosity of 385 SUS at 100° F., an acid number of 6, a specific gravity of 1.08 at 25° C., and a mixed aniline point of 61° F.

Staybelite Ester 5 (Hercules, Inc.) is a glycerol ester of hydrogenated rosin purified by steam distillation, typically having a softening point (Hercules drop method) of 81° C., an acid number of 5, a specific gravity of 1.06 at 25° C., and a mixed aniline point of 85° F.

Staybelite Resin (Hercules, Inc.) is hydrogenated rosin, typically having a softening point (Hercules drop method)

of 75° C., an acid number of 165, a saponification number of 167, a specific gravity of 1.045 at 25° C., and a mixed aniline point of 36° F.

Limited Poly-Pale Resin (Hercules, Inc.) is a reaction product of partially dimerized rosin and hydrated lime, typically having a softening point of 175° C. (Hercules drop method), an acid number of 63, a specific gravity of 1.10 at 25° C., and a mixed aniline point of 141° F.

Flexalyn (Hercules, Inc.) is a diethylene glycol ester of rosin, having a softening point (Hercules drop method) of 44° C., an acid number of 6, a specific gravity of 1.0 at 25° C., and a mixed aniline point of 76° F.

Pexate 510 E (Hercules, Inc.) is a high zinc content rosin-derived thermoplastic resin having a softening point of 118° C., a specific gravity of 1.16 at 25° C., a zinc content as zinc of 10.1%, and a mixed aniline point of 109° F. (theor.).

Permalyn 330 (Hercules, Inc.) is a glycerol ester of stabilized resin acids, typically having a softening point of 87° C. (Hercules drop method), an acid number of 7, a specific gravity of 1.06 at 25° C., and a mixed aniline point of 67° F. (theor.).

Surfactant AR-150 (Hercules, Inc.) is a medium chain length ethylene oxide adduct of rosin, typically having a viscosity of 400 centipoises at 25° C., and a specific gravity of 1.099 at 25° C.

Halowax 1014 (Koppers Co.) is a mixture of penta- and hexachloronaphthalene having about 62% chlorine, a hard amorphous waxy material typically having a softening point of 137° C., a viscosity of 35 SUS at 150° C., a maximum acid number of 0.05, and a specific gravity of 1.78 at 25° C.

Halowax 1001 (Koppers Co.) is a mixture of tri- and tetrachloronaphthalenes having about 50% chlorine, a hard amorphous waxy material melting to a very mobile liquid at 90-95° C., and having a viscosity of 30 SUS at 130° C., a maximum acid number of 0.05, and a specific gravity of 1.58 at 25° C.

Aluminum stearate No. 23 (Witro Chemical Co.) is a distearate made by the precipitation process from mixed fatty acids averaging 18 carbon atoms.

Polyvis O (Cosden Oil and Chemical Co.) is polyisobutylene, an oily liquid having an average molecular weight of about 400, a viscosity of 150 SUS at 100° F. and 42 SUS at 210° F., a specific gravity of 0.837 at 25° C., and an aniline point of 211° F. (straight).

Piccolastic A-50 (Pennsylvania Industrial Chemical Co.) is polystyrene having an average molecular weight of 350, a ball and ring melting point of 50° C., and a specific gravity of 1.04 at 25° C.

Piccoumaron 410L (Pennsylvania Industrial Chemical Co.) is a polyindene resin having a softening point of 100° C., a bromine number of 12, a melt viscosity of 100 centipoises at 175° C., and a mixed aniline point of 128° F.

Piccovar 450 (Pennsylvania Industrial Chemical Co.) is an alkyl-aromatic thermoplastic hydrocarbon resin having a large number of cyclic molecular structures. It has a softening point of 100° C., a maximum acid number of 1, a bromine number of 17, a melt viscosity of 100 centipoises at 185° C., a specific gravity of 1.05 at 25° C., and a mixed aniline point of 116° F.

Estynox 408 is iso-octyl epoxy stearate (Baker Castor Oil Co.). It has an iodine number of 2, a hydroxyl number of 4.8, a saponification number of 138, a specific gravity at 25° C. of 0.92, a viscosity of 18 centistokes at 25° C., and a mixed aniline point of 53° F.

The following examples illustrate various coating compositions according to the invention. It will be understood that the invention is not limited to the examples, which are merely illustrative, or to the materials, proportions, conditions, and procedures set forth therein. In the examples, the aniline points and viscosities refer to measurements on the plasticizer or mixture of plasticizers, and do not include the film-former or solvents.

**11**  
**EXAMPLE 1**

The following coating composition was applied from solution in solvent No. 1 to stencil base tissue, providing a total coated weight of 28 lbs. per 3,000 sq. ft.:

|                               | Volume percent | Parts by weight |
|-------------------------------|----------------|-----------------|
| <b>Material:</b>              |                |                 |
| CAB-500-1.....                | 14.3           | 16.7            |
| Hercolube D.....              | 21.2           | 21.6            |
| Hercolube A.....              | 25.3           | 25.3            |
| Celloylyn 21.....             | 11.1           | 11.7            |
| Mobilisol L.....              | 28.1           | 25.0            |
| Mixed aniline point, °F.....  | 95             |                 |
| Viscosity, cps. at 77° F..... | 97             |                 |

The Hercolube A in the composition is a low tack material contributing significantly to the lower tack of the plasticizing materials, minimizing blocking. The Celloylyn 21 serves to maintain stencil durability, while also contributing significantly to low oil transfer.

The stencil durability was rated good. The imaging speed, imaging quality, oil smudging and oil transfer were rated very good, and the blocking was rated good.

The plasticizing material when tested had a tack index of 11.5. When cooled from a melt, the coating composition formed an opaque, crumbly gel with no obvious oil separation.

**EXAMPLE 2**

The following coating composition was deposited from solution in solvent No. 2 to provide a total coated weight of 27 lbs. per 3,000 sq. ft.

|                               | Volume percent | Parts by weight |
|-------------------------------|----------------|-----------------|
| <b>Material:</b>              |                |                 |
| CAB 500-1.....                | 15.8           | 20.2            |
| Acetulan.....                 | 70.0           | 66.4            |
| Compressor Lube 1500.....     | 14.2           | 13.4            |
| Mixed aniline point, °F.....  | 70             |                 |
| Viscosity, cps. at 77° F..... | 14.5           |                 |

Acetulan is a low tack material providing a low tack plasticizing mixture. Inasmuch as the Acetulan has a low viscosity, a high viscosity mineral oil, Compressor Lube 1500 and a higher proportion of CAB 500-1 are employed to maintain stencil durability.

Stencil durability was rated good, imaging speed very good, imaging quality good, oil smudging very good, oil transfer good, and blocking fair.

When cooled from a melt, the coating composition formed a soft gel, with no pourable liquid.

**EXAMPLE 3**

The following coating composition was deposited from solution in solvent No. 3, to provide a total coated stencil weight 28 lbs. per 3,000 sq. ft.:

|                               | Volume percent | Parts by weight |
|-------------------------------|----------------|-----------------|
| <b>Material:</b>              |                |                 |
| CAB 500-1.....                | 14.3           | 16.7            |
| Hercolube A.....              | 25.9           | 25.9            |
| Stabelite ester No. 5.....    | 25.9           | 27.5            |
| Mobilisol L.....              | 34.0           | 30.2            |
| Mixed aniline point, °F.....  | 107            |                 |
| Viscosity, cps. at 77° F..... | 180            |                 |

The stencil durability was rated good; the imaging speed, fairly good; the imaging quality, very good; and the oil smudging, oil transfer and blocking properties, fair to good.

The plasticizing material when tested had a tack index of 12.4. When cooled from a melt, the coating composition was a viscous slush with small lumps, having no substantial amount of liquid which could be poured from the solid.

**EXAMPLE 4**

The following coating composition was deposited from solution in solvent No. 4, to provide a total coated weight of 28 lbs. per 3,000 sq. ft.

**12**

|                               | Volume percent | Parts by weight |
|-------------------------------|----------------|-----------------|
| <b>Material:</b>              |                |                 |
| CAB 500-1.....                | 14.3           | 16.9            |
| Hercolube A.....              | 31.4           | 31.7            |
| Abitol.....                   | 13.4           | 13.8            |
| Celloylyn 21.....             | 5.0            | 6.6             |
| Mobilisol L.....              | 35.9           | 32.4            |
| Mixed aniline point, °F.....  | 107            |                 |
| Viscosity, cps. at 77° F..... | 48             |                 |

10 The stencil durability was rated good; the imaging speed very good to excellent; the imaging quality very good to excellent; the oil smudging good, and the blocking good.

15 When cooled from a melt, the coating composition was a soft gel.

**EXAMPLE 5**

20 The following composition was deposited from solution in solvent No. 3, to provide a total coated weight of 26 lbs. per 3,000 sq. ft.:

|                               | Volume percent <sup>1</sup> | Parts by weight |
|-------------------------------|-----------------------------|-----------------|
| <b>Material:</b>              |                             |                 |
| CAB 500-1.....                | 17.6                        | 19.0            |
| Abitol.....                   | 22.2                        | 20.5            |
| Mobilisol L.....              | 60.2                        | 49.5            |
| Aluminum stearate No. 23..... | 130                         | 11.0            |
| Mixed aniline point, °F.....  |                             |                 |

<sup>1</sup> Exclusive of aluminum stearate.

30 The stencil durability was rated very good; the imaging speed on a roller copier good; the imaging quality on a roller copier very good; and the oil smudging, oil transfer, and blocking very good. In the absence of the stearate, oil smudging was fair and oil transfer very poor.

35 Other grades of aluminum stearate that may be employed include Witco grade 22 G, having a specific gravity of 1.01 at 25° C., a free fatty acid content of 6.1%, and a softening point of 157° C., the fatty acid content averaging less than 18 carbon atoms. Another suitable grade is Mallinckrodt grade AX. Both materials are distearates produced by the precipitation method.

**EXAMPLE 6**

40 The following coating composition was deposited from solution in solvent No. 1, to provide a coated weight of 27 lbs. per 3,000 sq. ft.:

|                              | Volume percent | Parts by weight |
|------------------------------|----------------|-----------------|
| <b>Material:</b>             |                |                 |
| CAB 500-1.....               | 14.3           | 18.35           |
| Modulan.....                 | 17.85          | 17.0            |
| Acetulan.....                | 67.85          | 64.70           |
| Mixed aniline point, °F..... | 55             |                 |

55 The stencil durability was rated fair; imaging speed very good, imaging quality good; oil smudging very good; oil transfer good; and blocking good.

**EXAMPLE 7**

60 The following composition was deposited from solution in solvent No. 5, to provide a total coated weight of 26.5 lbs. per 3,000 sq. ft.:

|                               | Volume percent | Parts by weight |
|-------------------------------|----------------|-----------------|
| <b>Material:</b>              |                |                 |
| CAB 500-1.....                | 14.3           | 15.6            |
| Hercolube A.....              | 41.0           | 38.6            |
| Halowax 1014.....             | 10.0           | 16.9            |
| Celloylyn 21.....             | 5.0            | 4.3             |
| Mobilisol L.....              | 29.7           | 24.6            |
| Mixed aniline point, °F.....  | 102            |                 |
| Viscosity, cps. at 77° F..... | 750            |                 |

75 The stencil durability was rated good; imaging speed very good; imaging quality very good, oil smudging and transfer good; and blocking very good.

The plasticizing materials were mutually soluble at elevated temperatures, but were found to contain undissolved Halowax 1014 at room temperature. All materials were soluble in the solvent. The coated stencil had a white cast apparently due to Halowax 1014 present in excess of its compatibility with the remaining plasticizing materials at room temperature. The performance char-

acteristics indicated that the Halowax 1014 functioned as a plasticizer during imaging while acting at least partially as a filler in the coating composition at room temperature.

The following Examples 8-12 show additional low oil transfer coating compositions according to the invention, applied similarly to the preceding examples:

## EXAMPLE 8

|                          | Example Number  |              |                 |               |                 |               |                 |               |                 |              |
|--------------------------|-----------------|--------------|-----------------|---------------|-----------------|---------------|-----------------|---------------|-----------------|--------------|
|                          | 8A              |              | 8B              |               | 8C              |               | 8D              |               | 8E              |              |
|                          | Vol.<br>percent | Wt.<br>parts | Vol.<br>percent | Wt.,<br>parts | Vol.<br>percent | Wt.,<br>parts | Vol.<br>percent | Wt.,<br>parts | Vol.<br>percent | Wt.<br>parts |
| <b>Material:</b>         |                 |              |                 |               |                 |               |                 |               |                 |              |
| CAB 500-1                | 14.3            | 16.3         | 14.3            | 16.7          | 14.5            | 16.7          | 14.3            | 16.9          | 14.3            | 16.8         |
| Hercolyn D               | 22.05           | 22.0         | 11.2            | 11.4          | 21.2            | 21.5          |                 |               | 21.2            | 21.4         |
| Staybelite ester No. 3   |                 | 15.0         | 16.2            |               |                 |               |                 |               |                 |              |
| Cellolyn 21              | 40.1            | 41.1         |                 |               |                 |               | 5               | 5.2           | 7.0             | 7.3          |
| Cellolyn 104             |                 |              |                 |               | 10.6            | 11.7          |                 |               |                 |              |
| Hercolube A              |                 | 31.4         | 31.2            |               | 25.4            | 25.2          | 31.4            | 31.6          | 14.7            | 14.8         |
| MCP-42                   |                 |              |                 |               |                 |               | 21.2            | 21.1          | 14.7            | 14.3         |
| MCP-99                   |                 |              |                 |               |                 |               |                 |               |                 |              |
| Mobilsol L               | 23.55           | 20.2         | 28.1            | 24.6          | 28.3            | 24.9          | 28.1            | 25.2          | 28.1            | 25.2         |
| Mixed aniline point, °F  | 85              |              | 97              |               | 103             |               | 100             |               | 104             |              |
| Viscosity, cps. at 77° F | 11,700          |              | 65              |               | 142             |               | 32              |               | 67              |              |

## EXAMPLE 9

|                          | Example Number  |              |                 |               |                 |               |                 |               |                  |              |
|--------------------------|-----------------|--------------|-----------------|---------------|-----------------|---------------|-----------------|---------------|------------------|--------------|
|                          | 9A              |              | 9B              |               | 9C              |               | 9D              |               | 9E               |              |
|                          | Vol.<br>percent | Wt.<br>parts | Vol.<br>percent | Wt.,<br>parts | Vol.<br>percent | Wt.,<br>parts | Vol.<br>percent | Wt.,<br>parts | Vol.,<br>percent | Wt.<br>parts |
| <b>Material:</b>         |                 |              |                 |               |                 |               |                 |               |                  |              |
| CAB 500-1                | 14.3            | 17           | 14.3            | 16.8          | 14.3            | 16.1          | 14.3            | 15.8          | 14.3             | 16.1         |
| Hercolyn D               |                 |              | 57.1            | 58.4          | 24.0            | 23.6          |                 |               | 21.2             | 20.8         |
| Cellolyn 21              |                 |              |                 |               | 18.9            | 21.0          | 18.9            | 20.8          | 5.0              | 5.1          |
| Pexate 510 E             |                 |              |                 |               |                 |               |                 |               |                  |              |
| Permalyn 330             |                 |              |                 |               |                 |               |                 |               | 24.8             | 25.1         |
| Hercolube A              | 57.2            | 58           | 28.6            | 24.8          | 24.0            | 23.1          | 27.6            | 26.3          | 25.0             | 24.1         |
| Modulan                  | 28.5            | 25           |                 |               |                 |               |                 |               |                  |              |
| Halowax 1001             |                 |              |                 |               |                 |               |                 |               | 6.4              | 9.8          |
| Mobilsol L               |                 |              |                 |               | 18.9            | 16.2          | 14.4            | 12.1          | 28.1             | 24.1         |
| Mixed aniline point, °F  | 86              |              | 82              |               | 90              |               | 92              |               | 95               |              |
| Viscosity, cps. at 77° F | 3,775           |              |                 |               | 500             |               | 5,125           |               | 57               |              |

## EXAMPLE 10

|                          | Example Number  |               |                 |               |                 |               |                 |               |                  |               |
|--------------------------|-----------------|---------------|-----------------|---------------|-----------------|---------------|-----------------|---------------|------------------|---------------|
|                          | 10A             |               | 10B             |               | 10C             |               | 10D             |               | 10E              |               |
|                          | Vol.<br>percent | Wt.,<br>parts | Vol.<br>percent | Wt.,<br>parts | Vol.<br>percent | Wt.,<br>parts | Vol.<br>percent | Wt.,<br>parts | Vol.,<br>percent | Wt.,<br>parts |
| <b>Material:</b>         |                 |               |                 |               |                 |               |                 |               |                  |               |
| CAB 500-1                | 15.8            | 20.3          | 14.3            | 18.3          | 14.3            | 17.0          | 14.3            | 18.0          |                  | 14.3          |
| CAB 451-1                |                 |               |                 |               |                 |               |                 |               |                  | 16.6          |
| Hercolyn D               |                 |               |                 |               | 56.8            | 58.6          |                 |               |                  |               |
| Hercolube A              |                 |               |                 |               |                 |               | 20.0            | 21.5          | 85.7             | 83.6          |
| Solulan 5                | 70.0            | 66.4          |                 |               |                 |               |                 |               |                  |               |
| Tridecyl alcohol         |                 |               | 38.5            | 35.6          |                 |               |                 |               |                  |               |
| Butyl stearate           |                 |               |                 |               |                 |               | 65.7            | 60.5          |                  |               |
| Polyvis O                |                 |               |                 |               | 28.8            | 24.4          |                 |               |                  |               |
| Mobilsol L               |                 |               | 47.2            | 46.1          |                 |               |                 |               |                  |               |
| Compressor lube 1500     | 14.2            | 13.3          |                 |               |                 |               |                 |               |                  |               |
| Mixed aniline point, °F  | 170             |               | 95              |               | 108             |               | 173             |               | 62               |               |
| Viscosity, cps. at 77° F | 290             |               |                 |               | 497             |               | 11.5            |               |                  |               |

<sup>1</sup>Theoretical.

## EXAMPLE 11

|                          | Example Number  |               |                 |               |                 |               |                 |               |                  |               |
|--------------------------|-----------------|---------------|-----------------|---------------|-----------------|---------------|-----------------|---------------|------------------|---------------|
|                          | 11A             |               | 11B             |               | 11C             |               | 11D             |               | 11E              |               |
|                          | Vol.<br>percent | Wt.,<br>parts | Vol.<br>percent | Wt.,<br>parts | Vol.<br>percent | Wt.,<br>parts | Vol.<br>percent | Wt.,<br>parts | Vol.,<br>percent | Wt.,<br>parts |
| <b>Material:</b>         |                 |               |                 |               |                 |               |                 |               |                  |               |
| CAB 500-1                | 14.3            | 18.4          | 14.3            | 17            | 14.3            | 17            | 14.3            | 18.8          | 14.3             | 17            |
| Solulan 5                | 85.7            | 81.6          |                 |               |                 |               |                 |               |                  |               |
| Ucon LB-70-X             |                 |               | 85.7            | 83            |                 |               |                 |               |                  |               |
| Ucon LB-300-X            |                 |               |                 |               | 86.7            | 83            |                 |               |                  |               |
| Hexadecyl alcohol        |                 |               |                 |               |                 |               | 85.7            | 81.2          |                  |               |
| Castor oil               |                 |               |                 |               |                 |               |                 |               | 85.7             | 83            |
| Mixed aniline point, °F  | <40             |               | 77              |               | 102             |               | 70              |               | 90               |               |
| Viscosity, cps. at 77° F |                 |               | 20              |               |                 |               | 40              |               | 720              |               |

## Example 12

| Example number            | 12A  | 12B   | 12C  | 12D   | 12E   | 12F   | 12G   | 12H   | 12J  |
|---------------------------|------|-------|------|-------|-------|-------|-------|-------|------|
| Material, volume percent: |      |       |      |       |       |       |       |       |      |
| CAB 500-1.....            | 14.3 | 14.3  | 14.3 | 14.3  | 14.3  | 14.3  | 14.3  | 14.3  | 14.3 |
| Hercolyn D.....           | 13.4 |       |      |       |       |       | 23.93 |       |      |
| Cellolyn 21.....          | 6.0  |       |      |       |       |       | 23.92 |       |      |
| Hercolube A.....          | 12.9 | 42.85 | 45.7 | 42.85 | 28.74 |       |       |       |      |
| Mobilisol L.....          | 25.2 |       | 20   |       | 28.22 | 42.85 |       | 42.85 | 20   |
| Piccotex 75.....          | 28.2 |       |      |       |       |       |       |       |      |
| Piccomaroon 410L.....     |      | 42.85 | 20   |       |       |       |       |       |      |
| Piccovar 450.....         |      |       |      | 42.85 |       |       |       |       |      |
| Piccolastic A-50.....     |      |       |      |       | 28.74 |       | 42.85 |       |      |
| Tridecyl alcohol.....     |      |       |      |       |       | 42.85 |       |       |      |
| Limed polypale.....       |      |       |      |       |       |       | 18.92 |       |      |
| Staybelite resin.....     |      |       |      |       |       |       | 42.85 |       |      |
| Estynox 408.....          |      |       |      |       |       |       |       | 65.7  |      |

Other representative materials that may be employed similarly to Hercolube A, MCP-42, and MCP-99 in the foregoing examples include the mono-pentaerythritol tetra-ester of valeric acid; the 89% mono-pentaerythritol, 11% di-pentaerythritol tetra-ester of caproic acid; the 89% mono-pentaerythritol, 11% di-pentaerythritol tetra-ester of caprylic acid; and the di-pentaerythritol tetra-ester of caproic acid, in the same order of preference. Additional materials that may be similarly employed include trimethylol propane tripelargonate, mixed mono- and di-pentaerythritol tetra-esters of mixed C-7, C-8, 25 and C-10 alkanic acids, and mixed mono- and di-pentaerythritol tetracaprylate.

We claim:

1. A thermographic stencil sheet which comprises an ink-pervious base sheet, and an ink-impervious coating thereon of a heat-flowable composition of

(a) a resinous thermoplastic film-forming material comprising cellulose acetate butyrate, and  
 (b) an oily, substantially non-volatile plasticizing material having a tack index of at least about 10, and a maximum mixed aniline point of about 110° F., said plasticizing material being partially but incompletely compatible with said film-forming material, the amount of (a) being about 8-50% by weight based on the total amount of (a) plus (b),  
 said composition forming a homogenous single phase melt when heated and forming a solid-liquid two-phase mixture when cooled from the melt to room temperature, said composition having a minimum compatibility temperature of about 120° F., at least one phase of said mixture incorporating substantial proportions of both said film-forming material and said plasticizing material,  
 said mixture having a maximum pourable liquid volume of about one-fourth the volume of the solid phase,  
 said composition being soluble in a volatile solvent and forming a substantially homogeneous continuous imperforate coating when deposited from a solution thereof, and said coating being provided on said base sheet by deposition of said composition on the base sheet from a solvent solution thereof and removing solvent therefrom, the melting point of said coating being at least about 150° F., said coating further becoming flowable and irreversibly physically altered when heated to its melting point for forming ink permeable image areas in the cooled stencil sheet.

2. A stencil sheet as defined in claim 1 wherein said plasticizing material comprises a member selected from the group consisting of mineral oil, hexadecyl alcohol, polypropylene glycol monobutyl ether, polyoxyethylene ethers of lanolin alcohols, pentaerythritol tetra-esters of aliphatic acids having from 5 to 10 carbon atoms, and trimethylol propane tri-esters of aliphatic acids having from 5 to 10 carbon atoms.

3. A stencil sheet as defined in claim 2 containing, in proportions by weight of said composition, about 5-85% of said member selected from said group.

15 4. A stencil sheet as defined in claim 1 wherein said plasticizing material comprises a plurality of plasticizers including a plasticizer having a nucleus selected from the group consisting of



30 5. A stencil sheet as defined in claim 1 wherein said plasticizing material comprises a plurality of plasticizers including a lanolin sterol.

6. A stencil sheet as defined in claim 5 containing about 5-75% of said lanolin sterol, in proportions by weight of said composition.

35 7. A stencil sheet as defined in claim 1 wherein said plasticizing material comprises a plurality of plasticizers including a member selected from the group consisting of hydrogenated resin acids, esters of hydrogenated resin acids, esters of resin acids, hydroabietyl alcohol, and esters of hydroabietyl alcohol.

40 8. A stencil sheet as defined in claim 7 containing about 5-75% of said member selected from said group, in proportions by weight of said composition.

9. A stencil sheet as defined in claim 1 including in 45 said coating an aluminum stearate gelling agent for said plasticizing material in a proportion of about 1-15% by weight based on the total amount of (a) plus (b) plus said gelling agent.

10. In a method of making an imaged stencil sheet employing a thermographic stencil sheet which includes an ink-impervious layer of a heat-flowable composition, wherein image areas of the stencil sheet are subjected to heat generated in adjacent image areas of an original by infra red ray absorption to render the composition flowable in the stencil sheet image areas and the composition is caused to flow therefrom and thereby form corresponding ink-transmitting image openings in the stencil sheet, the improvement which comprises employing as said stencil sheet the stencil sheet of claim 1.

## References Cited

## UNITED STATES PATENTS

|           |         |                  |       |          |
|-----------|---------|------------------|-------|----------|
| 1,790,987 | 2/1931  | Horii            | ----- | 117-35.5 |
| 1,792,095 | 2/1931  | Horii            | ----- | 117-35.5 |
| 2,808,777 | 10/1957 | Roshkind         | ----- | 117-36.1 |
| 3,062,675 | 11/1962 | Shelfo           | ----- | 117-35.5 |
| 3,120,611 | 2/1964  | Lind             | ----- | 117-36.1 |
| 3,177,086 | 4/1965  | Newman et al.    | ----- | 117-36.1 |
| 3,250,637 | 5/1966  | Frasher et al.   | ----- | 117-35.5 |
| 3,368,989 | 2/1968  | Wissinger et al. | ----- | 117-36.1 |
| 3,446,662 | 5/1969  | Newman           | ----- | 117-36.1 |

MURRAY KATZ, Primary Examiner

U.S. Cl. X.R.

UNITED STATES PATENT OFFICE  
CERTIFICATE OF CORRECTION

Patent No. 3,704,155

Dated November 28, 1972

Inventor(s) Anderson, Bror E. and  
Schick, Margery L.

It is certified that error appears in the above-identified patent and that said Letters Patent are hereby corrected as shown below:

Column 2, line 69: Insert after "as" --abaca,--;  
5 12: Change "formng" to --forming--;  
5 57: Change "polyoxyethyelne" to  
--polyoxyethylene--;  
5 57: Delete "or" and insert in place thereof  
--of--;  
7 44: Change "th" to --the--;  
7 44: Change "previous" to --pervious--;  
8 52: Change "actate" to --acetate--;  
9 5: Change "capric" to --caproic--;  
9 7: Change "it" to --its--;  
9 60: Change "Celloyln" to --Cellolyn--;  
9 70: Change "distilation" to --distillation--;  
10 4: Change "Limited" to --Limed--;  
10 7: Delete the period (.) following "of", at  
the end of line;  
10 39: Change "Witro" to --Witco--;  
10 46: Change "anline" to --aniline--;  
11 42: After "1500" insert a comma (,);  
11 53: After "weight" insert --of--;  
11 62: Change "stensil" to --stencil--; and  
13 1: Change "matetrial" to --materials--.

Signed and sealed this 13th day of November 1973.

(SEAL)

Attest:

EDWARD M. FLETCHER, JR.  
Attesting Officer

RENE D. TEGTMAYER  
Acting Commissioner of Patents

**Disclaimer**

8,704,155.—*Bror E. Anderson, Arlington Heights and Margery L. Schick, Mount Prospect, Ill.* THERMOGRAPHIC STENCIL SHEET AND METHOD OF MAKING AN IMAGED STENCIL SHEET. Patent dated Nov. 28, 1972. Disclaimer filed Jan. 24, 1974, by the assignee, *Weber Marking Systems, Inc.*

Hereby disclaims the portion of the term of the patent subsequent to Nov. 28, 1989.

[*Official Gazette March 12, 1974.*]

**Corrected Disclaimer**

3,704,155.—*Bror E. Anderson, Arlington Heights, and Margery L. Schick, Mount Prospect, Ill.* THERMOGRAPHIC STENCIL SHEET AND METHOD OF MAKING AN IMAGED STENCIL SHEET. Patent dated Nov. 28, 1972. Disclaimer filed Jan. 24, 1974, by the assignee, *Weber Marking Systems, Inc.*

Hereby disclaims the portion of the term of the patent subsequent to Sept. 26, 1989.

[*Official Gazette May 6, 1975.*]